

Jan. 3, 1933.

P. H. GEIGER

1,892,832

PROCESS OF PREPARING UNI-DIRECTIONAL CURRENT CARRYING DEVICES

Filed Sept. 10, 1925



Fig. 1.



Fig. 2.



Fig. 3.

INVENTOR:

P. H. Geiger,  
BY A. D. Vermaill  
His ATTORNEY

## UNITED STATES PATENT OFFICE

PAUL H. GEIGER, OF WILKINSBURG, PENNSYLVANIA, ASSIGNOR TO THE UNION SWITCH & SIGNAL COMPANY, OF SWISSVALE, PENNSYLVANIA, A CORPORATION OF PENNSYLVANIA

## PROCESS OF PREPARING UNI-DIRECTIONAL CURRENT CARRYING DEVICES

Application filed September 10, 1925. Serial No. 55,523.

My invention relates to uni-directional current-carrying devices or asymmetrical units, that is, devices which offer a higher resistance to current flowing through them 5 in one direction than to current in the opposite direction. More particularly my invention relates to the process of preparing such devices.

The present application is a continuation in 10 part of my co-pending application, Serial #670482, filed Oct. 24, 1923, for "process of preparing uni-directional current-carrying devices", in so far as the subject matter common to the two is concerned.

15 I will describe one method of preparing such devices, and will then point out the novel features thereof in claims.

In the accompanying drawing, Fig. 1 is 20 a view showing, in elevation, one form of blank ready to be prepared as a uni-directional current-carrying device according to my invention. Fig. 2 is a view showing in 25 vertical section, a uni-directional current-carrying device as it would appear at one point in a process embodying my invention. Fig. 3 is a view showing a completed uni-directional current-carrying device constructed in accordance with my invention.

Similar reference characters refer to similar 30 parts in each of the three views.

Referring to the drawing, the reference character A designates a blank of suitable material such as copper. As shown, this blank is of circular configuration and is provided with a central aperture A<sup>1</sup>, although this particular form is not essential. The copper blank is chemically cleaned in a suitable manner, as by a sand blast, or by immersing it for an instant in a caustic solution such as an aqueous solution of sodium hydroxide or common lye and afterward washing in water to remove the cleansing agent. The blank is then heated in the presence of air, as in an electric furnace. If the temperature of the copper reaches approximately 1040° centigrade, the surface of the blank assumes a glazed appearance. The temperature of the blank should be so controlled that it is close to and preferably just 45 below this glazing temperature or, say 1015°

centigrade. The application of heat causes a layer of red oxide of copper, or cuprous oxide, to be formed on each side of the blank. This layer is of comparatively low resistance. The heating process is continued until the 55 cuprous oxide layer is sufficiently thick to be mechanically strong. During this process there is formed also a thin coating of black oxide of copper or cupric oxide, over the outside of the blank. This black oxide coating 60 has a comparatively high electrical resistance.

After a sufficient amount of oxide has been formed on the copper, the blank is transferred immediately to a second furnace which 65 is maintained at a temperature of about 600° centigrade. In the second furnace the blank gradually cools in the presence of air. I have discovered that this gradual cooling to an intermediate temperature materially improves 70 the asymmetrical properties of the device.

When the temperature of the blank has decreased to substantially the temperature 75 of the furnace the blank is removed from the furnace and suddenly cooled or "quenched", a preferred method of accomplishing this being to plunge the blank into a spray of cold water or a current of cold air. The blank now appears as in Fig. 2, in which A 80 is the copper blank, 1 and 1<sup>a</sup> are the two layers of cuprous oxide, and 2 and 2<sup>a</sup> are the coatings of black copper oxide which cover the blank, the oxide coatings being greatly magnified in thickness in this view. 85

It has been found that a blank prepared in this manner will have the characteristic of offering a great deal higher resistance to an electric current flowing from the metallic copper A to the oxide 1 or 1<sup>a</sup> than to current 90 flowing in the other direction.

Since the resistance of the block oxide is very high it is desirable to make electrical connection directly with the red oxide coating and with the copper. To accomplish 95 this result the black oxide is removed from one side of the blank, as at 2, by abrasion as with a gentle sand blast, or by some other means. Both the black oxide coating 2<sup>a</sup> and the red oxide coating 1<sup>a</sup> may be similarly 100

removed from the other side to permit connection with the copper member A. I have found it advantageous to apply powdered petroleum coke to the oxide coating at this stage to decrease contact resistance.

One convenient arrangement for connecting the device to an outside circuit is illustrated in Fig. 3. In this view the aperture A<sup>1</sup> of the copper disk A is provided with a bolt 6 which is insulated from the disk by means of an insulating sleeve 8. This bolt also carries two terminal plates 4 and 4<sup>a</sup> of some suitable electro-conducting material such as copper, one of these plates being disposed on each side of the disk A. A number of thicknesses of tinfoil or leadfoil 3 are interposed between each plate and the disk for the purpose of securing more perfect contact. This tinfoil is particularly desirable adjacent the oxide coating, but may be dispensed with on the other side of the disk. The bolt 6 is provided with a nut 6<sup>a</sup> for clamping the parts rigidly together, it being noticed that insulating washers 5 and 5<sup>a</sup> are interposed between the bolt head and the nut and the adjacent terminal plates to prevent short-circuiting the device. The connections to the external circuit may then be conveniently made by means of wires 7 and 7<sup>a</sup> attached to plates 4 and 4<sup>a</sup>, respectively. When assembled in the manner shown in the drawing the device will offer considerably higher resistance to current flowing from wire 7<sup>a</sup> to wire 7 than to current flowing in the opposite direction.

It has been found that in some cases the asymmetrical properties of the devices can be improved by repeating the heating process several times. In such cases the blank is oxidized, gradually cooled, and quenched as before, the black oxide removed, and the blank is then returned to the furnace for a second heating after which it is gradually cooled and quenched as before. After each quenching the black oxide is removed, and this process is repeated till the surfaces attain the desired characteristics, after which the device may be assembled as described hereinbefore.

Devices prepared in accordance with my invention may be used for numerous purposes, such for examples as charging storage batteries from alternating current sources, and operating direct current electrical instruments from sources of alternating current supply.

Although I have herein shown and described only one process for preparing uni-directional current-carrying devices embodying my invention, it is understood that various changes and modifications may be made therein within the scope of the appended claims without departing from the spirit and scope of my invention.

Having thus described my invention, what I claim is:

1. The process of preparing metal for use in a uni-directional current-carrying device which consists in heating a chemically clean blank of copper in the presence of air to form cuprous oxide on the blank, and quenching the blank.

2. The process of preparing metal for use in a uni-directional current-carrying device which consists in heating a copper blank in the presence of oxygen to form cuprous oxide thereon, and quenching said blank in water.

3. The process of preparing metal for use in a uni-directional current-carrying device which consists in cleaning a metallic blank, successively heating the blank a number of times to form cuprous oxide thereon, and quenching the blank after each heating.

4. The process of preparing metal for use in a uni-directional current-carrying device which consists in cleaning a copper blank, heating the blank in the presence of air to a temperature just below the glazing temperature to form cuprous oxide thereon, and quenching the blank.

5. In the process of preparing metal for use in a uni-directional current-carrying device the steps of cleaning a copper blank, heating the blank to form oxide thereon, gradually cooling the blank to an intermediate temperature, and quenching the blank.

6. In the process of preparing metal for use in a uni-directional current-carrying device the steps of heating a copper blank in air to form oxide thereon, gradually cooling the blank in air to an intermediate temperature, and quenching the blank in water.

7. In the process of preparing metal for use in a uni-directional current-carrying device the steps of heating a copper blank in the presence of air to a temperature just below the glazing temperature, gradually cooling the blank to an intermediate temperature, and quenching the blank.

8. In the process of preparing metal for use in a uni-directional current-carrying device the steps of heating a metallic blank to form oxide thereon, gradually cooling the blank to substantially 600° centigrade, and quenching the blank.

9. In the process of preparing metal for use in a uni-directional current-carrying device the steps of heating a copper blank to substantially 1015° centigrade, to form cuprous oxide thereon, gradually cooling the blank to an intermediate temperature, and quenching the blank.

10. In the process of preparing metal for use in a uni-directional current-carrying device the steps of heating a copper blank to substantially 1015° centigrade to form cuprous oxide thereon, gradually cooling the blank to substantially 600° centigrade, and then quenching the blank.

11. In the process of preparing metal for use in a uni-directional current-carrying device the steps of heating a copper blank to substantially 1015° centigrade to form 5 cuprous oxide thereon, gradually cooling the blank to substantially 600° centigrade in the presence of air, and then quenching the blank.

12. The process of preparing metal for use in a uni-directional current-carrying device 10 which consists in cleaning a copper blank, heating the blank in the presence of air to substantially 1015° centigrade to form an inner low resistance oxide coating and an outer high resistance oxide coating thereon, gradually 15 cooling the blank in air to substantially 600° centigrade, quenching the blank, removing both oxide coatings from a portion of the blank, removing only the high resistance oxide coating from other portions of 20 the blank, and applying finely divided carbon to said blank.

13. The process of preparing metal for use in a unidirectional current-carrying device which consists in heating a metallic blank to 25 form oxide thereon, and then quenching the blank from a temperature of about 600° centigrade.

14. The process of preparing metal for use in a unidirectional current-carrying device 30 which consists in heating a metallic blank to a forming temperature to produce oxide thereon, and then quenching the blank from a temperature substantially lower than the forming temperature.

35 15. The process of preparing metal for use in a unidirectional current-carrying device which consists in heating a metallic blank to a forming temperature to produce oxide thereon, and then quenching said blank when 40 the blank is at a temperature intermediate the forming temperature and the temperature of the quenching medium.

In testimony whereof I affix my signature.  
PAUL H. GEIGER.

45

50

55

60

65